

Patented Aug. 21, 1928.

1,681,509

# UNITED STATES PATENT OFFICE.

LEON R. WESTBROOK, OF CLEVELAND, OHIO, ASSIGNOR TO THE GRASSELLI CHEMICAL COMPANY, OF CLEVELAND, OHIO, A CORPORATION OF OHIO.

## CADMIUM PLATING.

No Drawing.

Application filed November 23, 1926. Serial No. 150,376.

This invention relates to the electrodeposition of cadmium and to a process and a composition for that purpose.

As is known, deposits of cadmium upon other metals, for instance iron and steel, such as may be produced by electrodeposition, possess admirable protecting properties, but considerable difficulty has been encountered in devising a satisfactory method 10 for producing cadmium deposits having certain desired characteristics, as for example hardness and denseness. Among the difficulties encountered may be mentioned, also, the apparent inability to avoid producing 15 dark deposits of cadmium when plating at current densities above about 10 to 15 amperes per sq. ft., even in the presence of an addition agent.

An object of the invention is to provide 20 a method whereby cadmium may be electroplated in the form of bright, hard, dense and smooth deposits at current densities up to and even exceeding 80 amperes per sq. ft.

The invention is based upon my discovery 25 of the fact that under the influence of small amounts of certain metals in the cadmium plating solution, or bath, the above object may be attained.

The invention more particularly relates to 30 the addition of small amounts of nickel to a cadmium cyanide plating bath.

By applying this discovery, cadmium platings may be produced which are sufficiently hard and dense to withstand the 35 ordinary buffing operation without detriment thereto, and which even when produced at current densities above those heretofore regarded as operative for the production of bright deposits, are of excellent brilliance 40 and color surpassing those hitherto obtainable at lower current densities.

Among those metals the presence of which in small amounts in the cadmium plating bath produces the above-mentioned effects 45 are: nickel, cobalt and copper. In general I prefer to make use of those metals of the iron group having an atomic weight greater than 58. It has been found that the presence of a small amount of nickel is particularly effective in this connection, 50 cadmium platings possessing some of the before-mentioned desirable characteristics having been produced in the presence of as little as 0.0001% of nickel, based on the weight of

the bath. For practical operations the 55 nickel content of the bath should be at least 0.001%, and I prefer to use about 0.01 to 0.03%. The relative concentration of the added metal may vary within wide limits. For example, in the case of nickel, I have 60 found that cadmium platings made from a double cyanide bath containing as much as 0.03% of nickel (based on the weight of the bath) have marked brilliance and denseness. Quantities of nickel equal to and even exceeding 65 0.10% of the weight of the bath have been used with good results.

The effect of increasing amounts of the metal in the bath is to greatly broaden the band of current densities over which a bright 70 cadmium plate may be obtained. For example, using 0.005% of nickel in the solution, bright platings may be secured up to 30 amperes per sq. ft. on the cathode, while equally bright platings may be obtained at 75 current densities up to 60 amperes per sq. ft. using 0.03% of nickel. This characteristic effect is all the more important in view of the fact that it is difficult to secure a bright, smooth deposit of cadmium from a cyanide 80 bath free from the before-mentioned metals at any current density, and especially difficult at current densities exceeding about 10 amperes per sq. ft.

The effect of the added metal may be explained as being in part catalytic, in that 85 cadmium platings made from a bath containing lower amounts of the added metal contain no trace of that added metal, and in part an alloying effect, in that cadmium platings made from a bath containing relatively high amounts of the added metal have been found to contain a portion of the added metal in the form of an alloy. For example, in cadmium platings made from a double 90 cyanide bath containing 0.03% of nickel (based on the weight of the bath) there have been found small amounts of nickel in the form of a cadmium-nickel alloy. By the addition of larger amounts of the metal to 100 the cadmium plating bath there may be obtained alloy deposits having various desirable characteristics.

That the effect of the added metal may be in part catalytic may be still further substantiated by the observation that certain other metals, for example, arsenic, antimony, tin and thallium, appear to exert a 105

detrimental effect in the cadmium plating bath, analogous to the "poisoning" effect of arsenic in other catalytic operations.

The above-described characteristic effects are obtained by the addition of a small amount of the metal to any double cyanide cadmium solution, irrespective of its particular composition, and with or without the addition of ammonia or ammonium salts, caustic soda or sodium salts such as sodium sulfate. Preferably there may be present in the solution a so-called "addition agent" such as for example, gulac (the dry residue of the evaporation of sulfite cellulose waste liquor), dextrine, starch, or the like. The addition of the metal may be effected by adding a salt thereof, as for example, a sulfate or cyanide to the cadmium plating bath, or it may be introduced to the extent desired into cadmium hydroxide during preparation of the same and prior to the production of the bath.

The following examples illustrate, but do not limit, my invention:

25

*Example 1.*

To a bath prepared by dissolving 1.2 kgms. of cadmium hydroxide, 2.6 kgms. of sodium cyanide and 280 gms. of gulac in 30 20 liters of water, there is added 0.25 gm. of nickel as nickel cyanide. Cadmium platings obtained therefrom, at a current density of about 15 amperes per sq. ft., are bright, hard, dense and of good color.

35 Equally good platings may be obtained from the above solution at current densities up to about 60 amperes per sq. ft. by increasing the amount of the nickel there present to about 7.5 grams.

40 Good platings also may be obtained from the above solution by substituting for the nickel about from 12 to 35 grams of cobalt, in the form of a soluble salt thereof.

45

*Example 2.*

1.134 kgms. of cadmium hydroxide are combined with an amount of nickel hydroxide equivalent to about from 0.3 to 8.2 gms. of nickel, and dissolved in 22.7 liters of 50 water, preferably containing about 2% of  $\text{NaOH}$ , with 2.41 kgms. of sodium cyanide, 850 gms. of ammonium sulfate, and 255 gms. of gulac. Cadmium platings obtained from this solution at current densities of 55 from 15 to 60 amperes per sq. ft. are smooth, hard and dense; capable of withstanding buffing operation and have a desirable brilliance and good color.

From the foregoing description it is apparent that the relative proportions of the constituents in the cadmium plating baths may be varied, and the added metal may be incorporated in the solution in any suitable manner and at any suitable point in 65 the operation, without departing from my

invention. For example, a dry mixture, suitable for shipment and storage, comprising all of the ingredients of the solution, less the necessary water, may be prepared. Or the electroplater may be supplied with a dry mixture comprising, for instance, cadmium hydroxide, the added metal, in the form of a compound thereof, and gulac with directions as to the quantity thereof to be dissolved in a given quantity of water along with sodium cyanide and, if desirable, sodium hydroxide, separately supplied.

The electroplating from cadmium plating baths containing small amounts of a suitable added metal may be carried out substantially as disclosed in U. S. Patent No. 1,564,413, to Clayton M. Hoff; e. g., at room temperature using a potential of 4 to 6 volts, and preferably using cadmium anodes with an anode surface area equal to two or three times the cathode surface area. Known expedients such as agitation or circulation or heating or cooling of the bath, rotation of the electrodes, etc., may be employed.

90 I claim:

1. A cadmium plating bath for the electrodeposition of bright, hard, dense, smooth deposits of cadmium, the essential metal components of which bath consist of a cadmium compound and a substantial predetermined small amount of a compound of a metal of the iron group having an atomic weight greater than 58.

2. A cadmium plating bath for the electrodeposition of bright, hard, dense, smooth deposits of cadmium, the essential metal components of which bath consist of a cadmium compound and a substantial predetermined small amount of a compound of nickel.

3. A cadmium plating bath for the electrodeposition of bright, hard, dense, smooth deposits of cadmium, the essential metal components of which bath consist of a cadmium compound and a compound of nickel in an amount equal to about from 0.001% to 0.10% of the weight of said bath.

4. A cadmium plating bath for the electrodeposition of bright, hard, dense, smooth deposits of cadmium, the essential metal components of which bath consist of a cadmium compound and a compound of nickel in an amount equal to about from 0.01% to 0.03% of the weight of said bath.

5. As an electrolyte for the electrodeposition of bright, hard, dense, smooth deposits of cadmium, an aqueous solution comprising a compound of cadmium as the major metal component, a cyanide and a substantial predetermined small amount of a compound of a metal of the iron group having an atomic weight greater than 58.

6. As an electrolyte for the electrodeposition of bright, hard, dense, smooth deposits

70

75

80

85

90

95

100

105

110

115

120

125

130

of cadmium, an aqueous solution comprising a compound of cadmium as the major metal component, a cyanide and a substantial predetermined small amount of a compound of 5 nickel.

7. As an electrolyte for the electrodeposition of bright, hard, dense, smooth deposits of cadmium, an aqueous solution comprising a compound of cadmium as the major metal 10 component, a cyanide and about from 0.001% to 0.10% a compound of nickel based upon the weight of the solution.

8. As an electrolyte for the electrodeposition of bright, hard, dense, smooth deposits 15 of cadmium, an aqueous solution comprising a compound of cadmium as the major metal component, a cyanide, and about from 0.01% to 0.03% of a compound of nickel based upon the weight of the solution.

20 9. A cadmium plating bath for the electrodeposition of bright, hard, dense, smooth cadmium deposits, the essential metal components of which bath consist of a cadmium compound and a relatively small amount of 25 a compound of a metal of the group consisting of cobalt, nickel and copper.

10. As an electrolyte for the electrodeposition of bright, hard, dense, smooth cadmium deposits, an aqueous solution comprising 30 a cadmium compound, a cyanide and a relatively small amount of a compound of a metal of the group consisting of cobalt, nickel and copper.

11. A cadmium plating composition comprising a cadmium compound and a relatively small amount of a brightening agent, said brightening agent being a compound of 35 a metal of the group consisting of nickel, cobalt and copper, said metal compounds being

soluble in an aqueous alkali metal cyanide 40 solution.

12. A cadmium plating composition comprising a cadmium compound and a relatively small amount of a brightening agent, said brightening agent being a compound of 45 a metal of the iron group having an atomic weight greater than 58, said metal compounds being soluble in an aqueous alkali metal cyanide solution.

13. A cadmium plating composition comprising cadmium hydroxide and a relatively small amount of a brightening agent, said brightening agent being a nickel compound which is soluble in an aqueous alkali metal 50 cyanide solution.

14. A cadmium plating composition comprising cadmium hydroxide, an organic addition agent, at least one additional electrolyte and a relatively small amount of a brightening agent, said brightening agent 55 being a nickel salt which is soluble in an aqueous alkali metal cyanide solution.

15. A cadmium plating composition comprising about 50 parts of cadmium hydroxide, about 0.18 part of nickel as a compound 60 of nickel which is soluble in an aqueous alkali metal cyanide solution, about 38 parts of sodium sulfate and about 11.5 parts of gulac.

16. A cadmium plating composition comprising about 50 parts of cadmium hydroxide, about 0.18 part of nickel as nickel sulfate, about 38 parts of sodium sulfate, about 11.5 parts of gulac and about 100 parts of sodium cyanide.

In testimony whereof, I affix my signature.

LEON R. WESTBROOK.